

## UNITED STATES PATENT OFFICE.

LOUIS S. WERTZ, OF SHAKER HEIGHTS, OHIO, ASSIGNOR TO THE WERTZ COMPANY, OF CLEVELAND, OHIO, A CORPORATION OF OHIO.

## PROCESS OF TREATING MASONRY SURFACES.

No Drawing.

Application filed October 9, 1928. Serial No. 140,680.

My invention relates to methods of waterproofing or resurfacing masonry walls, ceilings, floors, et cetera, such as concrete, cement, brick and stone walls. It may be applied to a 5 surface of any material which is not, per se, waterproof, and which has openings or pores and which is not capable of resisting the absorption or transmission of water therethrough.

10 This application is a continuation, in part, of my application Serial No. 75,131 filed December 12, 1925.

15 Iron in powdered form, or reduced to fine particles, has been employed to waterproof concrete surfaces, but heretofore, so far as known to me, it has either been mixed with the concrete, or has been applied to the surface in the form of a wash, e. g., by mixing finely divided iron in a solution of an oxidizing 20 accelerator, and applying the same with a brush. When mixed with the concrete the iron expands within the concrete upon its oxidation, which renders the concrete friable, as pointed out in the patent to Flesheim, No.

25 1,113,112. The other method of application heretofore employed, that is, the application by means of a brush, has many disadvantages. According to this method, powdered iron is placed in a bucket containing sal-ammoniac and water, the liquid acting as a 30 carrier for the iron in its application by means of a brush. As the liquid is used as a carrier for the iron to effect the application thereof to the surface to be treated it must be employed greatly in excess of the quantity 35 required for the most efficient chemical action. Chemical action begins at once in such a mixture, the iron undergoing a slow process of oxidation, but sufficiently rapid to be distinctly discernable in the discoloration of the 40 liquid. To prevent all the iron from settling to the bottom, the workman was instructed to frequently stir the mixture but on account of the relative weight of the iron it quickly settled to the bottom. If the process was begun 45 with the proper proportion of iron the tendency of the iron to settle to the bottom resulted in constant change in the proportions because the workman took the material from the top with a constant lessening of the liquid

constituent. With this constant change in proportions of ingredients the final result was a coating on the surface treated which differed at different points in quantity of iron applied and in color, and, because of 55 the constant chemical reactions, a difference in the condition of the iron applied. It was a common practice also to add water as the liquid constituent decreased, which decreased the proportion of oxidizing accelerator. Furthermore, when the ingredients are applied in this way and on account of the excess of liquid it forms a water seal over the particles of iron which prevents oxidation until the 60 surface water evaporates, and also closes up the pores in the surface treated and prevents the entrance of the iron at the very points where their presence is most effective. The type of waterproofing to which the methods above described relate, in order to be effective, depends upon the oxidation of the material after it is in place, and especially upon the expansion of the iron by oxidation in the pores or voids. Therefore it is of great 70 importance not only to insert the iron particles fully into the voids, but to fill them uniformly over the entire surface and before the iron has been expanded by chemical action. 75

Therefore it is the object of this invention to more effectively and uniformly apply a 80 coating of the nature described and to effect such application at less expense than heretofore.

The invention consists of methods herein-after fully described and set forth in the appended claims.

The principal feature which characterizes my invention is the method of applying the oxidizable medium (preferably finely divided iron) to the surface to be treated. Instead of applying it to the surface with a brush or mixing it with the materials, I forcibly project it onto the surface whereby the particles are caused to enter fully into the pores. They are also projected into the pores in a substantially pure state, that is, before they have been partially chemically acted upon, or oxidized, and are so associated with the means for effecting oxidation that oxidation takes place with more rapidity than by methods hereto- 100

fore employed. The particles of iron expand within the pores to completely fill the same, yet without the tendency to render the material friable, as the expansion takes place 5 toward the open end of the voids after they have been completely filled.

A pneumatic gun is preferably employed to effect the forcible entry of the particles of iron into the pores, which may be of a construction 10 well known in the art; in this way air is used as a carrier for the iron instead of water, which is necessary for uniform and rapid oxidation.

In order that the particles of iron shall 15 oxidize quickly and effectively, they should be associated with water and air, and also an oxidizing accelerator, such as ammonium chloride (sal-ammoniac). Other oxidizing accelerators might be employed, for example, 20 other ammonium salts, sodium chloride, hydrochloric acid, alum and the like, but sal-ammoniac has been found particularly effective and well adapted to the purpose. The presence of these materials with iron in the 25 pores may be effected in various ways. One way of proceeding is to first wet the surface to be treated and then project onto the wet surface a dry mixture of iron (or other oxidizable medium) and sal-ammoniac (or other 30 oxidizable accelerator) in suitable proportion, as is well known in the art, a good proportion being 5% sal-ammoniac to 95% of iron. Or, as an alternative proceeding, a solution of sal-ammoniac and water might be applied to the 35 surface and the particles of iron be then projected onto the surface. A still different way of proceeding, and one which is hereinafter mentioned as the preferred method of carrying out my invention, is to project a mixture 40 of iron, sal-ammoniac, water and air onto the surface, either wet or dry. When this is done with a pneumatic gun the mixture of iron and sal-ammoniac will be projected through a nozzle and simultaneously mixed with water 45 flowing into the nozzle. The force (compressed air) which drives the mixture of iron and sal-ammoniac will thus supply the air needed in the mixture, and the quantity of water desired may be nicely regulated by 50 means of a suitable valve, and if additional air is needed it may be admitted at the nozzle, under control of a regulating valve. This is now considered the best way of applying these 55 materials.

When so applied all the elements are effectively associated with the iron to secure its oxidation, the water being in the form of a vapor or mist surrounding the particles of iron and trapped in the pores with the iron; 60 likewise the air is entrained by the solid particles of the mixture and so is brought into intimate contact therewith to most effectively secure the desired oxidation of the iron, and the quantities of water, oxygen (air), and 65 oxidizing accelerator may be nicely regulated

to secure the proper amount of each ingredient to secure the most effective oxidation.

As above indicated, if the surface to be treated is first wetted, the iron and sal-ammoniac may be applied in a dry condition, or 70 the sal-ammoniac may be first applied to the surface in the form of a solution, or all the materials may be applied at once to the surface when dry. In all of these methods of procedure the iron is forced into the pores in 75 the presence of water (in the liquid or vapor- ous state), air, and sal-ammoniac.

If, in any situation, it is not deemed necessary to secure rapid oxidation, the oxidizing accelerator may be omitted as an ingredient, 80 relying upon the slower oxidation by the surrounding air and by the air which enters the voids with the iron as a result of the described method of projecting it upon the surface being treated.

After the water has substantially evaporated from a surface treated as above described, it is preferable, in the absence of sufficient moisture in the air, to again treat the surface with water, either in the vaporous or 90 liquid form.

It is to be understood that the purpose of using water, in the above-described methods, is to effect the oxidation of the iron, assisted by the oxygen in the air; therefore whether 95 any water at all need be used, or the quantity to be used, will depend upon the moisture in the air surrounding the surface being treated, or the amount of moisture in the material itself.

If necessary, the surface to be treated may be first cleaned in any suitable manner, as for instance by means of a sand blast, the sal-ammoniac acting also as cleansing material.

My improved method applies a uniform 105 homogeneous mixture by means of compressed air which forces the oxidizable iron into the masonry voids, removing the excess water and supplying a large excess of moist air, thus preventing the formation of a water 110 seal over the iron particles. Such a water seal tends to prevent oxidation until the surface water evaporates and also tends to close up the voids and prevent the entrance of iron 115 to the places where its presence is most effective. I provide the necessary moisture but not to excess, and use air as the carrier. My method results in an accelerated oxidation of the iron and a complete filling of the voids by 120 the iron expansion, without the tendency to render the masonry friable, since the expansion takes place toward the open end of the voids after they have been filled completely. The result obtained is a wall structure having 125 a very even surface and which is capable of resisting the absorption of, or transmission of water therethrough.

What I claim is:

1. The process of waterproofing masonry surfaces which consists, in forcibly project- 130

ing into the masonry voids by compressed air, finely divided particles of iron mixed with water.

2. The process of waterproofing masonry surfaces which consists, in forcibly projecting into the masonry voids by compressed air, finely divided particles of iron mixed with water and an oxidizing accelerator.

3. The process of waterproofing masonry surfaces which consists, in forcibly projecting into the masonry voids by compressed air, finely divided particles of iron mixed with water and sal-ammoniac. <sup>10</sup>

Signed by me this 6th day of October, 1926.

LOUIS S. WERTZ.